

## UNITED STATES PATENT OFFICE

2,150,219

## ALUMINUM ALLOYS

Erik G. Grundstrom, Chicago, Ill., assignor to Advance Aluminum Castings Corp., Chicago, Ill., a corporation of Illinois

No Drawing. Application January 16, 1939,  
Serial No. 251,179

2 Claims. (Cl. 75—146)

The present invention relates to aluminum alloys.

More particularly the present invention relates to aluminum alloys of the non-tarnishable type.

The present invention is particularly applicable to aluminum alloys suitable for use as cooking utensils, which should not contain materials which might have a deleterious effect on foods cooked therein if absorbed by said foods.

10 An object of the present invention is to provide a non-tarnishable alloy which may be manufactured at relatively low cost.

A further object is to provide a non-tarnishable alloy which may be manufactured at low 15 cost and which is safe for use in cooking utensils.

Further objects will appear as the description proceeds.

The alloy according to the present invention contains the following materials within the percentages indicated:

|           | Per cent  |
|-----------|-----------|
| Zinc      | 1½ to 2½  |
| Magnesium | 2 to 3    |
| Silicon   | ¼ to ¾    |
| Aluminum  | Remainder |

25 A more specific formula within the ranges above indicated is the following:

|           | Per cent         |
|-----------|------------------|
| Zinc      | (approximate) 2  |
| Magnesium | (approximate) 2½ |
| Silicon   | (approximate) ½  |
| Aluminum  | Remainder        |

The percentages recited above are by weight.

The term "aluminum" as used herein is intended to cover commercial aluminum, which, as is well known, frequently contains impurities. In the accompanying claims, wherein the term "remainder aluminum" appears, it is to be understood that said remainder may include commercial impurities. 5

The alloy as above described is non-tarnishable, is corrosion resisting, and is safe for cooking 10 foods for human consumption.

What is claimed is:

1. An alloy suitable for use in cooking utensils comprising the following materials within the percentages indicated, by weight:

|           | Per cent     |
|-----------|--------------|
| Zinc      | 1½ to 2½     |
| Magnesium | 2 to 3       |
| Silicon   | ¼ to ¾       |
| Aluminum  | Remainder 20 |

2. An alloy suitable for use in cooking utensils comprising the following materials approximately according to the percentages indicated, by weight:

|           | Per cent     |
|-----------|--------------|
| Zinc      | 2            |
| Magnesium | 2½           |
| Silicon   | ½            |
| Aluminum  | Remainder 30 |

ERIK G. GRUNDSTROM.